

## UNITED STATES PATENT OFFICE

2,327,785

COMPOSITION OF MATTER AND METHODS  
AND STEPS OF MAKING AND USING THE  
SAMEMortimer T. Harvey, East Orange, N. J., assignor  
to The Harvel Corporation, a corporation of  
New JerseyNo Drawing. Application May 13, 1939,  
Serial No. 273,415

8 Claims. (Cl. 260—19)

The present invention relates generally to friction elements of the class of brake and clutch facings and the present invention relates more particularly to brake and clutch facings in which polymerizing and fatty oils are blended with phenol-aldehyde condensation reaction products which latter, in their intermediate states of condensation, are either soluble or intimately dispersible in said fatty oils and in which brake and clutch facings the blend has been cured by heating to carry on the phenol-aldehyde condensation reaction beyond the intermediate states and to polymerize or dry the fatty oil to produce dry, oil resistant products having friction characteristics advantageous to brake and clutch facings and having other advantageous characteristics such as infusibility at certain high temperatures and uniformity of frictional characteristics at high temperatures and under extreme changes of temperature and into which said brake and clutch facings said dry, oil resistant products are incorporated in the comminuted form.

Generally stated, the present invention relates to the formation of a friction producing material made with an oil soluble phenol resin and a glyceride oil brought to a stage of cure which can be ground to a granular size, or otherwise comminuted, and can be added to other ingredients commonly used in mixtures for forming brake linings and clutch facings, such as asbestos, rubber, carbon and so on.

In the practice of the present invention phenols are used which, upon condensation with a reactive methylene group supplying material, will produce a condensation product of resinous character which is soluble or intimately dispersible in fatty oils of polymerizing and drying character. The phenol and the reactive methylene group supplying material can be condensed first to an intermediate state and then blended with the fatty oil by dissolving or intimately dispersing and further condensed to a final state or curing with heat during which curing the fatty oil component of the blend is polymerized or dried whereby the entire blend becomes dry and resistant to the solvent action of oils and is in a state suitable for being comminuted by shredding, by grinding or by some other method.

Examples of the fatty oils suitable for use in the practice of the present invention are linseed oil, China-wood oil and soy bean oil and artificial oils made as by separating the glyceride radicles and fatty acids radicles of fatty oils and recombining these radicles to form other fatty oils. The fatty oils suitable for use in the practice of the present

invention are called herein, fatty oils which can be polymerized or dried.

Examples of the reactive methylene group supplying material suitable for use in the practice of the present invention are formaldehyde, para-formaldehyde, paraaldehyde, hexamethylene tetramine, acetaldehyde and furfuraldehyde.

Examples of phenols which upon condensation with a reactive methylene group, form condensation products soluble or intimately dispersible or miscible with fatty oils, are the tertiary alkyl phenols, e. g., para tertiary butyl phenol, para tertiary amyl phenol, the two para tertiary hexyl phenols, para phenyl phenol, the ortho phenols corresponding to those phenols above mentioned, carvacrol, xylenols, para cresol, mixtures of para cresol with ortho cresol and meta cresol and commercial phenols and mixtures of phenols which upon condensation with a reactive methylene group give oil soluble condensation product, cashew nut shell liquid, marking nut shell liquid, Japanese lac, and their several characteristic phenolic components and derivatives such as anacardic acid, cardol, anacardol, urushiol, cardanol and other similar phenols found in or derived from the plants of the Anacardiaceae family, and phenols generally which have unsaturated hydrocarbon side chains and which, with a reactive methylene group, give condensation products soluble in or dispersible with fatty oils and curable therewith to a dry, oil resistant form which can be produced in a final comminuted form. The phenols suitable for the practice of the present invention are classed herein as those phenols which have at least one of the readily reactive positions (ortho and para) unoccupied and which have a hydrocarbon substituent or substituents on the nucleus which give the phenol the characteristics of being soluble in oils and of forming aldehyde condensation products soluble or dispersible in oils and particularly in fatty oils of the kind described above. Other phenols suitable for use in the practice of the present invention have at least two of the readily reactive positions (ortho and para positions) unoccupied and some have all three of the readily reactive positions (the para and both of the ortho positions) unoccupied.

The characteristics of heat resistance, heat conductivity, non-softening under heat and resistance to water, oil and chemicals and especially uniformity of frictional characteristics over a wide range of temperature make the various products of cashew nut shell liquid suitable for use in friction elements. Also, the characteristic which

polymerized cashew nut shell liquid has of miscibility with rubber, phenolic resins, and other resins natural and artificial, pitches, gums and drying oils is advantageous in making up friction elements of various kinds and for various uses. And the reactions of polymerized cashew nut shell liquid with driers and with condensation materials, for example those having a methylene group such as formaldehyde and paraform, are advantageous for the handling and preparation of the intermediate and final products.

Other materials can be used with the modified cashew nut shell liquid and can be added before or after the modification process and also can be produced simultaneously with the modification such for example as in the case of producing a phenol-formaldehyde reaction product simultaneously with the production of a cashew nut shell liquid formaldehyde reaction product such as is disclosed in Patent Number 1,725,797. Drying oils, natural and artificial resins, gums, pitches, waxes, rubber, the polyhydric alcohol-polybasic acid type of resins, cellulose esters, sulphur, and so on can also be used with the modified cashew nut shell liquid or to produce the modification of the cashew nut shell liquid with or without the aid of heat, and with or without increase or decrease in pressure. Also ethers, esters, hydrogenation products, and so on of cashew nut shell liquid can be used. Another form of modified cashew nut shell liquid suitable for the purposes of the present invention is produced from the decarboxylated product called cardanol which can be obtained by distilling cashew nut shell liquid preferably at a low pressure (about 10 millimeters of mercury) or by distilling with steam to remove the carbon and oxygen atoms of the carboxyl group of the anacardic acid ingredients of the cashew nut shell liquid and to separate other ingredients. Cardanol can be modified to the dry, infusible state in a number of ways such as those described above for cashew nut shell liquid itself. Further, numerous combinations of the methods disclosed and referred to above can be used to modify cashew nut shell liquid and derivatives thereof to a dry, infusible state to produce various materials suitable for the various purposes of the present invention and to suit the various conditions under which friction elements are used. Also the residue obtained by distilling cashew nut shell liquid, as with steam or under vacuum, to obtain cardanol is suitable as a phenol for the practice of the present invention. This residue can be, for example, from forty per cent to sixty per cent, more or less, of the cashew nut shell liquid subjected to distillation. In some cases this residue is used as obtained, in other cases this cashew nut shell liquid residue is polymerized before or during the process of practicing the method of the present invention.

The present application is a continuation in part of my copending application Serial Number 46,743, filed October 25, 1935, issued to Patent Number 2,165,140, July 4, 1939, and of all that part of said copending application which describes or refers to the use of oil soluble phenol-aldehyde (reactive methylene group) condensation products with polymerizing and drying fatty oils to obtain dry, oil resistant brake linings and clutch facings.

Illustrative examples of mixtures of friction materials containing the blends of oil soluble phenol-aldehyde condensation products or resins

and polymerizing and drying fatty oils of the present invention are given below.

*Example A*

5 A quantity of cashew nut shell liquid is heated with about five per cent of its weight of concentrated sulphuric acid and about fifteen per cent of the weight of the cashew nut shell liquid of water, with rapid stirring to disperse the sulphuric acid thoroughly and quickly throughout the cashew nut shell liquid. The heating of this mixture is carried to about 300° F. to about 350° F. Up to this point the material is a thick liquid polymer and is identified herein as material of Example A. During this process certain metals which occur naturally in cashew nut shell liquid are precipitated as sulphate salts and these salts can be separated from the treated cashew nut shell liquid by filtering while the cashew nut shell liquid is still in a comparatively thin liquid state, and can be done expeditiously by adding the sulphuric acid in two substantially equal increments with the filtering in between the treatments with the two increments in which case the water also is divided into two substantially equal increments. This metal freed material is also identified herein as material of Example A.

*Example B*

30 (a) To one mole of para tertiary butyl phenol, about two moles of formaldehyde (in about 40% solution in water) are added, with a sodium hydroxide solution as a catalyst, and left to stand for about five days at room temperature, after which the mixture is neutralized and the resin is dehydrated. To one part by weight of this resin, about two parts by weight of China-wood oil are added and the mixture heated up to between 450° F. to 550° F. in the manner of preparing a varnish to get a body. This heating is continued until the body is quite heavy but still pourable at temperatures convenient for handling. The heavy bodied resin-China-wood oil mixture is then poured, while hot, into shallow pans to a depth of about three or four inches and cured in an oven at about 325° C. for about sixteen hours. The resin-China-wood oil product, when cool, is solid but just slightly resilient and can be shredded or comminuted into small particles.

35 (b) Instead of two parts by weight of China-wood oil to one of the resin above, one part of China-wood oil is added and the mixture bodied and cured in a manner substantially the same as set forth above. This resin-China-wood oil product is solid and somewhat brittle and can be comminuted to fine particles.

40 (c) The proportion of resin to China-wood oil can be varied between and outside of the limits bounded by the ratios set forth in Example B (a) and (b) to obtain final comminuted products of various consistencies. Also to vary the desired consistency the temperatures and duration of bodying and curing can be varied. And also to obtain various consistencies linseed oil or soy bean oil or other polymerizing or drying glyceride oils, can be used in place of all or part of the China-wood oil.

*Example C*

45 About four hundred parts by weight of the cashew nut shell liquid distillation residue described above, taken as it comes from the still or, if cold, heated to about 300° F. to make it flow-

able, is strained through a screen to remove any lumps or solid particles and at about 200° F. mixed with one hundred parts of China-wood oil, and with about ten parts of diethyl sulphate and about two and one-half parts of furfuraldehyde, the mixture being thoroughly stirred and poured into shallow pans and cured for about sixteen hours at about 275° F. This material when cold is comminuted to small particles. The quantity of furfuraldehyde can be increased to about twenty-five parts, in the formula last given above, to obtain a hard, brittle resin which is pulverized.

*Example D*

About two hundred parts by weight of the cashew nut shell liquid distillation residue hereinabove described and one hundred parts of the liquid material of Example A, above are heated together at about 280° F. and thoroughly mixed with one hundred and fifty parts of China-wood oil, about six parts of diethyl sulphate and twenty-five parts of furfuraldehyde and cured and comminuted as in Example C.

*Example E*

About equal parts by weight of cardanol, phenol (carbolic acid) and a 37% solution of formaldehyde are heated, with ammonia as a catalyst, under a reflux condenser for about one hour, after which the resulting resin is separated from the water while hot and dehydrated. About four parts of this resin, eight parts of bodied linseed oil, forty-eight parts of cashew nut shell liquid residue, one part of diethyl sulphate and three parts of furfuraldehyde are melted together, by first heating the resin, bodied linseed oil and cashew nut shell liquid residue at about 260° F. to about 300° F. and then adding the diethyl sulphate and furfuraldehyde at about 180° F., and thoroughly intermixed, after which the mixture is cured in shallow pans at about 275° F. for about sixteen hours. The cured material is comminuted or pulverized.

The cardanol of this last example and methods of producing it are described in my Patent Number 2,098,824, issued November 9, 1937.

*General example*

A general illustrative example of a brake lining or clutch facing composition made up of any of the comminuted phenolic resin-glyceride oil materials described above as illustrative examples or of any mixture of any two or more of them is as follows. Seventy-five parts of asbestos, in the form known in the brake lining manufacturing field as "long fiber asbestos," from ten to fifteen parts of a binder, and from fifteen to ten parts of the selected comminuted phenolic resin-glyceride oil material are thoroughly intermixed, molded to shape and cured to modify the binder to a dry state. The binder can be rubber, a phenolic resin, a drying oil or any combination thereof, examples being well known in the brake and clutch manufacturing field and in the patent art. Any of the phenolic resins described above as suitable for making the comminuted material of the present invention, when in an intermediate state of condensation, with or without a polymerizing or drying glyceride oil, can be used as the binder and, in addition to being a binder, will serve with the comminuted material and the asbestos as a frictional functioning part of the brake lining or clutch facing. For further illustrative examples of brake lining and clutch

facing compositions using the comminuted material of the present invention, that is, comminuted, dry material made from a blend of a phenol-aldehyde resin and a drying or polymerizing glyceride oil, reference is hereby made to the disclosure in my copending application Serial Number 37,749, filed August 24, 1935, to Patent Number 2,164,326, issued July 4, 1939, of which the present application is a continuation-in part, and particularly to the general and specific examples of the composition of the comminuted material described therein and of the brake lining and clutch facing compositions made up of said comminuted material and to the last paragraph of the specification of said copending application.

Having thus described my invention, what I claim is:

1. A composition of matter, capable of augmenting the frictional characteristics of a friction element, comprising a substantially dry and infusible composition obtained by heat converting to a substantially dry and infusible material, a mixture of a heat polymerizable oil, a dialkyl sulphate, furfuraldehyde and a product selected from the group consisting of cashew nut shell liquid and residue of cashew nut shell liquid obtained by distilling cashew nut shell liquid until the quantity by weight of the residue is between about 40 to 60% of the quantity by weight of said cashew nut shell liquid.
2. A composition of matter, capable of augmenting the frictional characteristics of a friction element, comprising a substantially dry and infusible composition obtained by heat converting to a substantially dry and infusible material, a mixture of a heat polymerizable oil, a dialkyl sulphate, furfuraldehyde and a product selected from the group consisting of cashew nut shell liquid and residue of cashew nut shell liquid obtained by distilling cashew nut shell liquid until the quantity by weight of the residue is between about 40 to 60% of the quantity by weight of said cashew nut shell liquid, the quantity of said product being materially greater than that of said furfuraldehyde.
3. A composition of matter, capable of augmenting the frictional characteristics of a friction element, comprising a substantially dry and infusible composition obtained by heat converting to a substantially dry and infusible material, a mixture of a heat polymerizable oil, diethyl sulphate, furfuraldehyde and a product selected from the group consisting of cashew nut shell liquid and residue of cashew nut shell liquid obtained by distilling cashew nut shell liquid until the quantity by weight of the residue is between about 40 to 60% of the quantity by weight of said cashew nut shell liquid.
4. A composition of matter, capable of augmenting the frictional characteristics of a friction element, comprising a substantially dry and infusible composition obtained by heat converting to a substantially dry and infusible material, a mixture of a heat polymerizable oil, diethyl sulphate, furfuraldehyde and a product selected from the group consisting of cashew nut shell liquid and residue of cashew nut shell liquid obtained by distilling cashew nut shell liquid until the quantity by weight of the residue is between about 40 to 60% of the quantity by weight of said cashew nut shell liquid, the quantity of said product being materially greater than that of said furfuraldehyde.
5. A composition of matter, capable of aug-

menting the frictional characteristics of a friction element, comprising a substantially dry and infusible composition obtained by heat converting to a substantially dry and infusible material, a mixture of diethyl sulphate, furfuraldehyde, a heat polymerizable oil, and residue of cashew nut shell liquid obtained by distilling cashew nut shell liquid until the quantity by weight of the residue is between about 40 to 60% of the quantity by weight of said cashew nut shell liquid, the quantity by weight of said residue being greater than the quantity by weight of either said aforementioned other substances and the quantity by weight of said oil being greater than the quantity by weight of either said first two mentioned substances.

6. A composition of matter, capable of augmenting the frictional characteristics of a friction element, comprising a substantially dry and infusible composition obtained by heat converting to a substantially dry and infusible material, a mixture of a heat polymerizable oil, diethyl sulphate, furfuraldehyde and residue of cashew nut shell liquid obtained by distilling cashew nut shell liquid until the quantity by weight of the residue is between about 40 to 60% of the quantity by weight of said cashew nut shell liquid, the ratio of the quantity by weight of said residue to the quantity by weight of said oil being about 4 to 1, the ratio of the quantity by weight of said oil to the quantity by weight of said diethyl sulphate being about 10 to 1 and the quantity by weight of said oil being greater than the quantity by weight of said furfuraldehyde.

7. A composition of matter, capable of aug-

menting the frictional characteristics of a friction element, comprising a substantially dry and infusible composition obtained by heat converting to a substantially dry and infusible material, a mixture of diethyl sulphate, furfuraldehyde, China-wood oil and residue of cashew nut shell liquid obtained by distilling cashew nut shell liquid until the quantity by weight of the residue is between about 40 to 60% of the quantity by weight of said cashew nut shell liquid, the quantity by weight of said residue being greater than the quantity by weight of either said aforementioned other substances and the quantity by weight of said oil being greater than the quantity by weight of either said first two mentioned substances.

8. A composition of matter, capable of augmenting the frictional characteristics of a friction element, comprising a substantially dry and infusible composition obtained by heat converting to a substantially dry and infusible material, a mixture of China-wood oil, diethyl sulphate, furfuraldehyde and residue of cashew nut shell liquid obtained by distilling cashew nut shell liquid until the quantity by weight of the residue is between 40 to 60% of the quantity by weight of said cashew nut shell liquid, the ratio of the quantity by weight of said residue to the quantity by weight of said oil being about 4 to 1, the ratio of the quantity by weight of said oil to the quantity by weight of said diethyl sulphate being about 10 to 1 and the quantity by weight of said oil being greater than the quantity by weight of said furfuraldehyde.

MORTIMER T. HARVEY.